

# UNITED STATES PATENT OFFICE.

ARNOLD MCKERROW, HARRY WALTON, AND GEORGE ERNEST SHEARSMITH, OF MANCHESTER, ENGLAND, ASSIGNEES TO DRAKE PRINTING COMPANY, LIMITED OF MANCHESTER, ENGLAND.

## METHOD OF MAKING TRANSFERS.

1,161,711.

Specification of Letters Patent. Patented Nov. 23, 1915.

No Drawing.

Application filed February 23, 1915. Serial No. 10,112.

*To all whom it may concern:*

Be it known that we, ARNOLD MCKERROW, HARRY WALTON, and GEORGE ERNEST SHEARSMITH, subjects of the King of Great Britain and Ireland, and residents of Blake street, Hulme, Manchester, in the county of Lancaster, England, have invented certain new and useful Improvements in Methods of Making Transfers, of which the following is a specification.

This invention relates to transfers of the kind described in the specification of U. S. Patent No. 1030908 and has for its object to improve upon such transfers so that they can be readily and efficiently transferred to printed or dyed goods and so that the transferred design is unaffected by the pattern or color of the goods upon which it is placed.

Our invention comprises the provision upon the design which is printed upon a carrying body from which it is detached by heat, of both an opaque layer or covering and an adhesive coating, the latter being of such a nature that it melts by heat but rests upon the surface of and does not penetrate or sink into the adjacent color layers.

In one convenient application of our invention, we provide the design upon the transfer sheet in the manner described in the specification previously referred to, that is by giving the transfer sheet or carrying body a surface impermeable to wax, coating said sheet with a wax layer and printing the design upon the latter by surface printing means. We then coat the design with an opaque covering layer, such as Cremnitz white mixed with a slow drying oil. The said covering forms a solid groundwork or base for the design when it is subsequently transferred to printed or dyed goods so that the pattern or color of the latter does not interfere with the design. The opaque covering is allowed to dry and harden and when practically dry is printed or varnished with an adhesive coating which melts by

heat. By reason of the preliminary drying of the opaque covering, the adhesive coating rests in a film upon the latter and does not penetrate or sink into the colors of the design.

The adhesive coating may comprise gum dammar dissolved in turpentine with or without the addition of gum thus which acts to render the coating more pliable. A suitable mixing is:—2 ounces gum dammar, 1 ounce gum thus, 3 ounces turpentine.

When it is desired to transfer the design to a printed or dyed fabric or other material, the adhesive coating is placed upon the fabric, and a heated iron or the like applied to the back of the carrying body. The adhesive layer then attaches itself to the fabric and draws the design from off the fusible layer upon the carrying body.

With our improved transfer, the adhesive coating in conjunction with the opaque layer insure the effectual transference of the design with a suitable ground to the printed or dyed goods.

Our transfers may be employed for placing designs on fabrics, wood, glass, leather or other materials.

Having now described our invention, what we claim as new and desire to secure by Letters Patent is:—

1. The process of producing transfers for use in transfer printing by heat alone, consisting in providing a support or carrying body with a surface impermeable to wax, coating the said surface with an easily melting material, printing a design upon said coating by means of surface printing, covering said design with an opaque groundwork, and printing a fusible adhesive coating upon said opaque covering, as set forth.

2. The process of producing transfers for use in transfer printing by heat alone, consisting in providing a support or carrying body with a surface impermeable to wax, coating the said surface with an easily melting material, printing a design upon said

coating by means of level printing means, covering said design with an opaque covering of Cremnitz white mixed with a slow drying oil, and when said covering is nearly dry, printing thereon a fusible adhesive coating of gum dammar, gum thus and turpentine, as set forth.

In testimony whereof we have signed our

names to this specification in the presence of two subscribing witnesses.

ARNOLD MCKERRROW.

HARRY WALTON.

GEORGE ERNEST SHEARSMITH.

Witnesses:

ARTHUR HUGHES.

GEORGE WEAVER.